

## UNITED STATES PATENT OFFICE

2,113,810

## SULPHURIZED OILS

Bert H. Lincoln and Waldo L. Steiner, Ponca City,  
Okla., assignors to Continental Oil Company,  
Ponca City, Okla., a corporation of Delaware

No Drawing. Application December 28, 1936,  
Serial No. 117,900

## 5 Claims. (Cl. 87—9)

Our invention relates to sulphurized oils and more particularly to lubricants containing a specific class of sulphur containing compounds. This application is a continuation in part of our copending application, Serial No. 11,588, filed March 18, 1935.

In our said copending application, we have disclosed an improved type of sulphurized oil prepared by adding to a hydrocarbon oil a dihydric or monohydric ester of an unsaturated organic acid, which ester has been sulphurized. In said application, the value of a sulphurized oil made in accordance with our application for use in cutting lubricants, extreme pressure lubricants and crank case lubricants was pointed out. Sulphurized oils, made by adding sulphurized glycerides or sulphurized vegetable or animal oils to lubricants, have long been known but these oils do not possess the advantages of oils compounded by the use of sulphurized dihydric and monohydric esters. The advantage of oils compounded with monohydric or dihydric esters arises from the fact that no derivatives of glycerine are present, which derivatives will break down, liberating glycerine which is easily polymerized or oxidized. The presence of glycerine, therefore, will cause gumming and sludging, which is deleterious, especially in case of internal combustion engines where high temperatures and pressures are involved, which will readily facilitate gumming and sludging.

Lubricating oils prepared with monohydric and dihydric esters have the further advantage of being less viscous than those prepared by sulphurized glycerides. Moreover the viscosity does not increase as rapidly on long time heating with sulphurized monohydric and dihydric ester. This is very important in commercial lubricants.

Higher speeds and greater bearing pressures in modern internal combustion engines have made it necessary for automotive engineers to develop improved bearings. Modern bearings which have resulted from this improvement are of three general types, namely those comprising generally cadmium alloys, those comprising generally mixtures of copper and lead together with small amounts of other metals, and alloys containing a high percentage of lead. While these new bearing materials are capable of withstanding higher pressures and greater speeds than the old Babbitt bearings, they are more susceptible to corrosion, resulting from the action of oxidation products of the lubricants.

One object of our invention is to provide a sulphurized lubricant of inhibited corrosion prop-

erties with respect to the new type of "soft" metal bearings.

Another object of our invention is to provide a lubricant containing a small amount of a sulphurized monohydric or dihydric ester which lubricant will not be corrosive to bearings of the "soft" metal group, but which will, nevertheless, be sufficiently chemically active to precipitate objectionable compounds of such metals as sulphides.

Another object of our invention is to provide a lubricant possessing a high degree of oiliness.

Another object of our invention is to provide a lubricant which will possess a decreased rate of oxidation.

Another object of our invention is to provide a lubricant of minimized sludging characteristics.

Other and further objects of our invention will appear from the following description.

We have pointed out in our copending application, Serial No. 11,588 that the monohydric and dihydric esters of unsaturated fatty acids, when sulphurized, will yield products which may be added to a hydrocarbon oil to obtain an improved lubricant.

We have discovered that certain of the monohydric and dihydric esters, when prepared in a certain manner, are superior corrosion inhibitors and are therefore especially desirable for use with the new type "soft" metal bearings. Certain of these compounds falling within the generic class and prepared in accordance with our invention have the further advantage that they are oxidation and sludging inhibitors.

We do not know the theory of the new effects produced. We believe, however, that the corrosion inhibiting and anti-oxidation effects of these monohydric and dihydric esters, prepared in a certain manner, may be explained. Most metals tend to act as catalysts, increasing the rate of oxidation. For example, when a hydrocarbon oil is heated in contact with air in the presence of copper, a sludge comprising hydrocarbon oxidation products will form much more rapidly than if the oil is heated to the same temperature in a glass container, out of contact with copper. This oxidation increasing effect of metals is true to various degrees for other metals. Soaps and oxides of such metals as calcium, cadmium and iron are catalysts in oxidation reactions for petroleum derivatives and are used, for example, in the preparation of fatty acids and other oxidation products from hydrocarbons. Sulphurized esters of our invention are strongly polar compounds and we believe they tend to form a pro-

5 tective layer over metallic parts, serving to insulate the metal from the main body of oil, thus inhibiting the oxidation catalytic effect of the metal. We believe, further, that traces of such metallic salts as do form, such as iron soaps, copper soaps, and cadmium soaps, which result from the reaction of the oxidized hydrocarbons with the metals are precipitated by the sulphur in our sulphuretted esters. The sulphides are insoluble 10 in hydrocarbon oil and are much poorer oxidation catalysts than the soaps and the metals themselves. By the formation of sulphides and their precipitation, the catalytic effect is decreased and the oxidation is minimized.

15 15 We have discovered that certain types of sulphurized esters are superior to others and that these could be most advantageously prepared in certain ways. This type consists of monohydric and dihydric esters, prepared from fatty oils in 20 which the linoleic or similar two double-bonded fatty acid content ranges from 10 to 60 per cent and in which the linolenic or similar three or more double-bonded fatty acid is present in quantities less than 5 per cent. Examples of fatty oils 25 in which the fatty acid content meets these requirements are as follows:

|                         | Per cent linoleic or two double-bonded acid | Per cent linolenic or three or more double-bonded acid |
|-------------------------|---------------------------------------------|--------------------------------------------------------|
|                         | Percent                                     | Percent                                                |
| 30                      |                                             |                                                        |
| 35 Rape seed oil.....   | 15                                          | 1                                                      |
| Arachis oil.....        | 21                                          | 0                                                      |
| Cottonseed oil.....     | 53.6                                        | 0                                                      |
| Maize oil.....          | 41.6                                        | 0                                                      |
| Ravison oil.....        | 27                                          | 2                                                      |
| Sunflower seed oil..... | 58.4                                        | 0                                                      |
| Soya bean oil.....      | 57.5                                        | 2.2                                                    |

40 40 Linseed oil, for example, would not meet the requirements, since its two doublebonded acid content is 62 per cent and its three or more doublebonded acid content is 24 per cent. Menhaden oil would not be available, since its per cent linoleic or two doublebonded acid content is 29.6 per cent, while its linolenic or three or more doublebonded acid content is 31 per cent.

45 45 The fatty oils of high unsaturation, as represented by linseed oil, menhaden oil, whale oil, and sperm oil, are unsatisfactory. These highly unsaturated oils form insoluble products upon being sulphurized. Then, too, they form tarry and gummy products when employed as lubricants. If the unsaturation, however, is reduced by hydrogenating or partially hydrogenating them to reduce the three or more doublebonded acid content but leaving a substantial percentage of linoleic or two doublebonded acid 50 content, then they may be satisfactorily used in our invention. The fatty oils or fatty acids of the single doublebond type such as oleic or erucic acids, yield sulphurized esters which are only partially satisfactory as oxidation and corrosion 55 inhibitors. We attribute this to the fact that they do not take up as much sulphur as fatty oils and fatty acids having a high percentage of two doublebonded or linoleic acid in which the sulphur which is taken up is more firmly held.

60 60 The result is that, if sulphurized esters are made from single doublebonded fatty acids a larger amount of inhibitor is required to stop corrosion, which results in a dark color for the blended lubricant. This dark color is objectionable from 65 a sales standpoint and, furthermore, the em-

ployment of a greater amount of inhibitor is expensive.

65 In preparing our inhibitors, fatty oils of the type described are applicable to our invention, that is, those having a high acid content of the two doublebonded acid type while having a small linolenic acid content. The oils are first converted into the corresponding dihydric or mono-hydric ester in any suitable manner, for example, the oil may be refluxed with an equal volume 10 of the desired monohydric or dihydric alcohol containing three per cent of dry hydrochloric acid for several hours. On cooling the alcohol-glycerol layer is separated and the refluxing operation repeated. This procedure converts all 15 of the original glycerides into the desired alcohol ester and, at the same time, eliminates most of the unsaponifiable matter in the whole oil. The ester is then water washed and dried. The esters, of course may be made by directly esterifying 20 the fatty acids. The esters alone or admixed with petroleum oil are heated to a temperature between 360° and 390° F., and from 5 per cent to 20 per cent or more of elemental sulphur is slowly stirred in until it is combined. When higher 25 percentages of sulphur are used, the temperature must be raised from 410° to 420° F. for a short period after the sulphur has apparently dissolved or combined. Sometimes it is desirable to continue this higher temperature range for a 30 period of about an hour. While adding the sulphur, care must be exercised to prevent the heat of reaction from raising the temperature appreciably above 400° F. This can be done by controlling the heating step, it being remembered 35 that the sulphur combining reaction is an exothermic one. Temperatures outside the range of 360° to 390° F. may be used but we find the results are not as good as when the temperature range mentioned is employed. Higher or lower 40 temperatures may be employed by varying the time of heating. The sulphurized esters may be refined to improve their color, by treatment with activated clay or carbon or by using fuller's earth, silica gel, bentonite, and other decolorizing methods. 45

45 Inhibitors thus prepared may be added to hydrocarbon oils in amounts from .01 per cent to 5 per cent by weight. Amounts in excess of 5 per cent may be added without injury, but it does not appear that any further results will be achieved by adding greater amounts. 50

50 A machine for testing corrosiveness of lubricating oils on soft metal bearings employed by us consists of four connecting rods provided with a 55 four speed lubrication arrangement. The soft metal bearings were employed on the shaft and connecting rod bearings. The crank shaft was turned at a speed of 1,250 R. P. M. The connecting rods lay flat and the piston ends were 60 free to rub upon an iron plate. Two quarts of oil were used in the lubricating system and the temperature was maintained at 350° F. The test was run for twenty-two hours.

65 A high grade ordinary hydrocarbon lubricating oil was tested in the machine above described and it was found that, for a cadmium alloy bearing and a copper lead bearing, a loss of over one gram per bearing insert was experienced. The oil contained 14.6 per cent of sludge. The same oil was then blended with two tenths of one per cent of a sulphurized ester of linoleic acid, that is, a sulphurized ester made from an organic acid, having a high linoleic acid content and a comparatively low linolenic acid content, and con- 70 75

taining 15 per cent by weight of sulphur. This blend was then tested upon the same machine and under the same conditions. It was found that the corrosion per bearing insert on both the cadmium 5 alloy bearing insert and the copper lead bearing insert was about .06 of a gram per bearing insert and the oil contained only 5.2 per cent of sludge.

Another apparatus for measuring the corrosion tendencies of lubricating oils, under conditions 10 approximating use, is the "Underwood" machine, which was developed by the General Motors research department and is described in their literature and is known to those skilled in the art. In this machine, jets of oil under pressure of ten 15 pounds per square inch are directed at half bearing inserts in the presence of air, the oil being held at a temperature of 325° to 350° F. The test is usually run for about five hours.

A well refined hydrocarbon lubricating oil containing .05 of one per cent of lead oxide in the 20 form of lead naphthenate was tested. The lead naphthenate was employed to speed up the rate of corrosion and thereby shorten the time required for the test. Using this blend without any 25 corrosion inhibitor, there was .570 mg. loss on the copper lead alloy and 1710 mg. on the cadmium alloy. Another portion of the same lubricating oil containing .05 of one per cent of lead oxide in the form of lead naphthenate was then blended 30 with .2 of one per cent of sulphurized methyl esters of corn oil fatty acids containing 15 per cent sulphur. The test on the Underwood apparatus was repeated under exactly the same conditions. It was found that the loss of metal from 35 corrosion for a copper lead bearing alloy was 60 mg. and for a cadmium alloy only 10 mg.

Another blend was made from another portion of the same test oil base, that is, the hydrocarbon oil containing .05 of one per cent of lead oxide in 40 the form of lead napthene with a sulphurized ester of oleic acid, namely sulphurized methyl oleate containing 20 per cent sulphur. .2 of one 45 per cent of the sulphurized methyl oleate was used in making the blend. The loss on the copper lead bearing was 500 mg. and the loss on the cadmium alloy was 1590 mg.

It will be observed that the tests, (which are merely representative of many which were conducted) clearly show the improved results produced by our sulphurized esters of high linoleic 50 acid content without a correspondingly high linolenic acid content.

In the preparation of our inhibitors, we find that better results are obtained if the amount of sulphur employed approximates two atoms per 55 molecule of fatty acid ester. The heating period of 410° to 420° F. is continued just long enough to give .1 per cent blend in a lubricating oil which will not appreciably darken a copper strip at 60 210° F. at 30 minutes. An inhibitor prepared in the manner just described, that is with approximately two atoms of sulphur per molecule of fatty acid ester, when tested on the Underwood apparatus, using the same test base oil, that is, 65 a hydrocarbon oil containing lead oxide in the form of lead naphthenate, which blend contained .1 of one per cent of a sulphuretted methyl ester of soya bean oil containing 18 per cent of sulphur

gave a corrosion loss on the copper lead alloy bearing insert of only 10 mg. and on the cadmium alloy bearing insert of 20 mg.

It will be understood that the amount of inhibitor to be used in making a blend with a hydrocarbon oil depends on a number of factors such as the type of crude oil used in manufacturing the hydrocarbon oil, the manner and degree of refining and the conditions of use. In general, a range from .01 of one per cent to 5 per cent by 10 weight of sulphurized ester will be sufficient for all practical purposes.

It will be understood that our inhibitors may be applied to other lubricants besides hydrocarbon oils. They may be employed for example in 15 greases which are hydrocarbon oils, thickened with soaps. It will be understood that certain features and sub-combinations are of utility and may be employed without reference to other features and sub-combinations. This is contemplated by and is within the scope of our claims. It is further obvious that various changes may be made in details within the scope of our claims without departing from the spirit of our invention. It is, therefore, to be understood that 20 our invention is not to be limited to the specific details shown and described.

Having thus described our invention, what we claim is:

1. A lubricant comprising in combination a 30 major proportion of a hydrocarbon oil and a minor proportion of a sulphurized monohydric or dihydric ester of linoleic acid.

2. A lubricant comprising in combination a major proportion of hydrocarbon oil and a minor 35 proportion of sulphurized monohydric or dihydric ester of organic acids, the glycerides of which are present in natural oils, said organic acids having a high percentage of linoleic acid and low percentages of linolenic acid.

3. A lubricant comprising in combination a hydrocarbon oil and from .01 to 5 per cent of a sulphurized monohydric or dihydric ester obtained by esterifying fatty acids derived from naturally occurring glycerides which contain from 45 60 to 10 per cent of glycerides of linoleic acid and less than 5 per cent of glycerides of linolenic acid with a monohydric or dihydric alcohol.

4. A lubricant comprising in combination a major proportion of a hydrocarbon oil and a 50 minor proportion of a sulphurized, monohydric or dihydric ester of linoleic acid the glyceride of which is present in oils selected from the following group: rape seed oil, arachis oil, cottonseed oil, maize oil, ravigon oil, sunflower seed oil, soya 55 bean oil.

5. A lubricant comprising in combination a major proportion of a hydrocarbon oil and a minor proportion of a sulphurized, monohydric or dihydric ester of linoleic acid the glyceride of 60 which is present in oils selected from the following group: rape seed oil, arachis oil, cottonseed oil, maize oil, ravigon oil, sunflower seed oil, soya bean oil, said sulphurized esters containing from 5 per cent to 20 per cent by weight of elemental 65 sulphur.

BERT H. LINCOLN.  
WALDO L. STEINER.